

## UNITED STATES PATENT OFFICE.

HUBERT A. MYERS, OF TOLEDO, OHIO, ASSIGNOR TO THE HUBERT A. MYERS COMPANY, OF TOLEDO, OHIO, A CORPORATION OF OHIO.

## METAL MOLD.

No Drawing.

Application filed January 14, 1922. Serial No. 529,381.

To all whom it may concern:  
Be it known that I, HUBERT A. MYERS, a citizen of the United States, and a resident of Toledo, in the county of Lucas and State 5 of Ohio, have made an Invention Appertaining to Metal Molds; and I do hereby declare the following to be a full, clear, and exact description of the invention, such as will enable others skilled in the art to 10 which it appertains to make and use the same.

The object of my invention is to provide an efficient permanent iron mold or mold containing iron that may be readily constructed and shaped and wherein smooth, perfect metal castings may be formed. My invention particularly has for its object to 15 form a machinable alloy or mixture containing iron for molds that may be used for rapidly casting metals, particularly ferrous metals, over a long period without deterioration of the molds.

In order that iron molds for casting metals, particularly ferrous metals, may be durable, they should be formed of an iron low 20 in silicon and carbon. Otherwise the silica at the surface will be fused by the repeated application of the heat of molten metal and cause pitting of the surface of the matrix. 25 Also high carbon iron will not withstand the constant or rapid changes in temperature that such molds are subjected to without warping or cracking. Low silicon and low carbon iron, however, are difficult to work 30 and machine. Furthermore, iron molds may be treated or lined with materials, to protect them from the effect of heated metals, which treatments sometimes cause slight softening of the molding surface.

These objectionable features I have overcome by forming a mixture or alloy of low carbon and low silicon iron, a small amount of manganese, not to exceed 2% of manganese, which greatly reduces injurious thermal effects produced by temperature changes, such as that caused by rapid expansion and contraction, and a small amount of nickel, not to exceed 20%, which operates to soften the iron so as to make it shapable 45 or machinable and at the same time stiffens the surface as against any action of the lining or surfacing material that may be used to protect the surface of the mold from the molten metal inserted in the mold. If desired, the manganese may be omitted, but I

find it preferable to use the small amount of manganese designated.

In forming the molds embodying my invention I make a mixture or an alloy, which is hereinafter described broadly as an alloy, 60 of nickel and low carbon and low silicon iron, using a relatively small amount of nickel in the alloy. Probably the best results are obtained when the amount of the nickel is not less than 5% and not more than 65 15%. However, fairly good results are obtained by alloy formed of from 1% to 20% of nickel and the balance of iron. To this may be added about 1% of manganese. As much as 2% may be used. The molten metal 70 is then poured and shaped in the manner well known in the art to form a matrix and a connecting sprue hole.

The nickel operates to stiffen or strengthen the iron while the manganese prevents warping of the mold.

The invention is particularly advantageous when the surfaces of the matrices are treated with zinciferous materials that may be used to prevent adherence of the metal 80 castings, particularly ferrous metal castings, and to form smooth, perfect castings. The zinc tends to weaken the iron at the surface when the iron is repeatedly treated with the materials and heated in the casting operations. The zinciferous materials will, however, not effect the nickel but will adhere to 85 the iron and form a protective surfacing material. The zinc is held or absorbed or attracted by the iron of the alloy, while at 90 the same time the nickel strengthens the molds at the surfaces of the matrices.

I claim:

1. A mold for casting metals containing nickel and iron in alloyed relation. 95
2. A mold for casting metals formed of an alloy containing nickel and iron.
3. A mold for casting metals and containing iron and from 5% to 15% of nickel.
4. A mold for casting metals and containing from 1% to 20% of nickel and iron. 100
5. A mold for casting metals formed of an alloy containing nickel and iron, the surface of the matrix of the mold covered with a zinciferous material. 105
6. A mold for casting metals formed of an alloy containing nickel and iron, the surface of the matrix of the mold covered with a zinciferous material.
7. A mold for casting metals and contain- 110

ing iron and from 5% to 15% of nickel, the surface of the matrix of the mold covered with a zinciferous material.

8. A mold for casting metals and containing of from 1% to 20% of nickel and iron, the surface of the matrix of the mold covered with a zinciferous material.

9. A mold for casting metals formed of an alloy containing nickel and low carbon and silicon iron.

10. A mold for casting metals formed of an alloy containing nickel and low carbon and silicon iron.

11. A mold for casting metals and containing low carbon and silicon iron and from 5% to 15% of nickel.

12. A mold for casting metals and containing of from 1% to 20% of nickel and low carbon and silicon iron.

20 13. A mold for casting metals formed of an alloy containing nickel and low carbon and silicon iron, the surface of the matrix of the mold covered with a zinciferous material.

25 14. A mold for casting metals formed of an alloy containing nickel and low carbon and silicon iron, the surface of the matrix of the mold covered with a zinciferous material.

30 15. A mold for casting metals and containing low carbon and silicon iron and from 5% to 15% of nickel, the surface of the matrix of the mold covered with a zinciferous material.

35 16. A mold for casting metals and containing of from 1% to 20% of nickel and low carbon and silicon iron, the surface of the matrix of the mold covered with a zinciferous material.

40 17. A mold for casting metals formed of an alloy containing nickel, iron, and a small amount of manganese.

45 18. A mold for casting metals formed of an alloy containing nickel, iron, and a small amount of manganese.

19. A mold for casting metals and containing iron, from 5% to 15% of nickel, and a small amount of manganese.

50 20. A mold for casting metals and containing of from 1% to 20% of nickel, a small amount of manganese, and the balance of low carbon iron.

21. A mold for casting metals formed of an alloy containing nickel, iron and a small

amount of manganese the surface of the 55 matrix of the mold covered with a zinciferous material.

22. A mold for casting metals formed of an alloy containing nickel, iron, and a small amount of manganese, the surface of the 60 matrix of the mold covered with a zinciferous material.

23. A mold for casting metals and containing iron and from 5% to 15% of nickel, and from  $\frac{1}{2}\%$  to 2% of manganese, the surface of the 65 matrix of the mold covered with a zinciferous material.

24. A mold for casting metals and containing of from 1% to 20% of nickel, and from  $\frac{1}{2}\%$  to 2% of manganese, and iron, the 70 surface of the matrix of the mold covered with a zinciferous material.

25. A mold for casting metals formed of an alloy of nickel, low carbon and low silicon iron, and a small amount of manganese. 75

26. A mold for casting metals formed of an alloy containing nickel, low carbon and low silicon iron, and a small amount of manganese.

27. A mold for casting metals and containing low carbon and low silicon iron, from 5% to 15% of nickel, and a small amount of manganese. 80

28. A mold for casting metals formed of an alloy of nickel, low carbon and low silicon iron, and a small amount of manganese, the surface of the matrix of the mold covered with a zinciferous material. 85

29. A mold for casting metals formed of an alloy containing nickel, low carbon and low silicon iron, and a small amount of manganese, the surface of the matrix of the mold covered with a zinciferous material. 90

30. A mold for casting metals and containing low carbon and low silicon iron, and from 5% to 15% of nickel, and from  $\frac{1}{2}\%$  to 2% of manganese, the surface of the 95 matrix of the mold covered with a zinciferous material.

31. A mold for casting metals and containing of from 1% to 20% of nickel and from  $\frac{1}{2}\%$  to 2% of manganese, and the balance of low carbon and low silicon iron, the surface of the matrix of the mold covered with a zinciferous material. 100

In testimony whereof, I have hereunto signed my name to this specification.

HUBERT A. MYERS.